# EUROPEAN PATENT SPECIFICATION

(11) **EP 0 198 401 B1**
(45) Date of publication and mention of the grant of the patent: **19.07.1989**
(21) Application number: 86104816.3
(22) Date of filing: 09.04.1986
(51) Int. Cl.: D21H 5/20

(54) **New water-dispersible synthetic fiber**
Wasserdispergierbare Synthesefaser
Fibre synthétique dispersible dans l'eau

(30) Priority: 09.04.1985 US 721346
(43) Date of publication of application: 22.10.1986
(73) Proprietor: E.I. DU PONT DE NEMOURS AND COMPANY, Wilmington Delaware 19898 (US)
(72) Inventor: Shiffler, Donald Albert, Kinston North Carolina 28501 (US)
(74) Representative: Abitz, Walter, Dr.-Ing.

(56) References cited:
- FR-A- 2 124 574
- US-A- 3 249 669
- US-A- 3 416 952
- US-A- 4 297 414
- JAPANESE PATENTS GAZETTE, week E40, 17th November 1982, page 7, Derwent Publications Ltd., London, GB; & JP - A - 57 139 600 (TEIJIN) 28-08-1982
- JAPANESE PATENTS GAZETTE, week 8403, 29th February 1984, page 8, Derwent Publications Ltd., London, GB; & JP - A - 58 208 500 (TEIJIN) 05-12-1983

## Description

This invention concerns new water-dispersible synthetic polymer fiber, particularly of poly(ethylene terephthalate), and its preparation.

### Background of invention

There has been increased interest in recent years in water-dispersible synthetic fiber, especially of polyester. Such water-dispersible fiber is used in various non-woven applications, including paper-making and wet-laid non-woven fabrics, sometimes as part of a blend, often with large amounts of wood pulp, or fiberglass, but also in applications requiring only polyester fiber, i.e., unblended with other fiber. This use, and the requirements therefor, are entirely different from previous more conventional use as tow or staple fiber for conversion into textile yarns for eventual use in woven or knitted fabrics, because of the need to disperse this fiber in water instead of to convert the fiber into yarns, e.g., by processes such as carding, e.g. in the cotton system. It is this requirement for water-dispersibility that distinguishes the field of the invention from previous, more conventional polyester staple fiber.

Most such water-dispersible polyester fiber is of poly(ethylene terephthalate), and is prepared in essentially the same general way as conventional textile polyester staple fiber, except that most water-dispersible polyester fiber is not crimped, whereas any polyester staple fiber for use in textile yarns is generally crimped while in the form of tow, before conversion into staple fiber. Thus, water-dispersible polyester fiber has generally been prepared by melt-spinning the polyester into filaments, combining the filaments to form a tow, drawing, applying a suitable coating to impart water-dispersible properties, generally in the same way as a finish is applied to a tow of conventional textile filaments, and then, generally without any crimping (or with imparting only some mild wavy undulations in some cases to provide extra bulk and a three-dimensional matrix), converting the tow into staple. Some prior polyester staple fiber has been prepared in uncrimped form, e.g., for use as flock in pile fabrics, but for such use, water-dispersibility has not been required.

Polyester fibers are naturally hydrophobic, so it is necessary to apply to the polyester a suitable coating, as disclosed by Ring et al. in U.S. Patent No. 4,007,083, Hawkins in U.S. Patent Nos. 4,137,181, 4,179,543 and 4,294,883, and Viscose Suisse in British Patent No. 958,430, to overcome the inherent hydrophobic character of the polyester fiber without creating foam or causing the fibers to flocculate. It is this coating that has distinguished water-dispersible polyester fiber from more conventional polyester staple fiber, rather than any inherent characteristic feature of the polyester itself, or of its shape, such as the cross-section. Heretofore, so far as is known, the cross-section of all commercial water-dispersible polyester fiber has been round. Indeed the cross-section of most commercial polyester staple fiber has generally been round, because this has been preferred.

Although, hitherto, most synthetic polymeric water-dispersible fiber has been formed of polyester, being inexpensive and plentiful, increasing amounts of polyolefins and polyamides are beginning to be used for water-dispersible fibers, and so the invention is not limited only to polyesters, but covers other synthetic polymers.

### Summary of invention

According to the present invention, there is provided new synthetic polymer water-dispersible fiber, especially polyester fiber, characterized in that the fibers are of cruciform cross-section.

A cruciform cross-section has been used heretofore for other polyester fibers, as described herein. Other than the cross-section, the water-dispersible fiber of the invention may be essentially similar to prior water-dispersible polyester or other synthetic polymer fibers, although the advantages described hereinafter may provide the opportunity for additional modifications. The invention will be described hereinafter with special reference to polyester fiber, although it will be recognized that other synthetic polymers, such as polyamides and polyolefins, may also be used.

The fibers of the invention may be made conveniently by melt-spinning and drawing polyester filaments of appropriate denier per filament (dpf), and applying thereto a suitable coating to impart water-dispersible characteristics. The filaments are then generally cut into staple of whatever length is desired for the end-use contemplated.

The use of a cruciform cross-section for the water-dispersible fiber of the invention has, surprisingly, been found to promote dispersibility, in comparison with a round cross-section, and this imparts to the resulting wet-laid fibers better uniformity, more opacity, good permeability, and an attractive flannel-like hand as will be seen in the Example.

### Brief description of drawings

Figure 1 shows a cruciform cross-section for a stylized fiber according to the invention.
Figure 2 shows a typical spinneret orifice for spinning filaments of the invention.

### Disclosure of the invention

As indicated above, a cruciform cross-section has already been used for more conventional polyester staple fiber, that has been spun into filaments and drawn, cut, converted into spun yarn, and used in woven or knitted fabrics. Such fiber did not have the water-dispersible characteristics required for this invention. Similarly, polyester filaments having a cruciform cross-section are already known from Lehmicke U.S. Pat. No. 2,945,739, which discloses a process for melt-spinning polyamide and polyester filaments of, inter alia cruciform cross-section, and woven and knitted fabrics from staple fibers, and from Jamisson U.S. Pat. No. 3,249,669, which discloses a process for making a multifilament yarn of polyester filaments of various cross-sections, including a cruciform cross-section. Oriented polyester filaments of non-round cross-section have also been described by Frankfort et al, in U.S. Pat. Nos. 4,134,882 and 4,195,051, having been prepared by spinning at a very high speed (6,000 ypm (5486 m/min)), which high speeds could also be used to prepare oriented polyester filaments of cruciform cross-section as a substrate for applying thereto a suitable coating to impart water-dispersible characteristics, and thereby obtain water-dispersible fiber according to the invention. None of this art concerns the field of the present invention. However, the polyester filamentary substrates for making the water-dispersible fiber of the invention may be prepared by the techniques described therein, or by appropriate modifications of these or other known techniques of making polyester filaments of non-round cross-section.

The prior art references disclose parameters for a cruciform cross-section and Figure 1 is essentially as shown therein.

The preparation of the polyester staple fiber is otherwise conventional, involving the steps of melt-spinning polymer into filaments, collecting the filaments into a tow, drawing the tow, and applying a suitable coating to impart water-dispersible characteristics. If low shrinkage is desired, the drawn filaments are generally annealed.

Selection of an appropriate coating to promote water-dispersibility is important, and more of such coating is generally required than for comparable weights of fiber of round cross-section of similar dpf, because of the larger surface area of the periphery of the cruciform cross-section. It is especially important to provide good boundary lubrication properties. For this reason, an ethoxylated coating is preferred.

Suitable coatings are disclosed in Hawkins, U.S. Pat. Nos. 4,137,181, 4,179,543 and 4,294,883 or a synthetic copolyester of poly(ethylene terephthalate) units and poly(oxyalkylene) of groups derived from a poly(oxyalkylene) glycol having an average molecular weight in the range of 300 to 6,000, as disclosed, e.g. in McIntyre, et al. U.S. Pat. Nos. 3,416,952, 3,557,039 and 3,619,269, referred to therein, other useful segmented copolyesters are disclosed in Raynolds U.S. Patent No. 3,981,807.

Such polyester fiber is generally prepared first in the form of a continuous filamentary uncrimped tow or, if extra bulk is required, and a more three-dimensional matrix, the filaments may be provided with mild wave-like undulations by a mild crimping-type process, and the uncrimped or mildly wave-like filaments are cut to the desired cut length, i.e. to form the water-dispersible fiber, which is generally sold in the form of bales, or other packages of cut fiber. Suitable cut lengths are generally from about 5 to about 90 mm (1/4 to 3 inches), generally up to 60 mm (2-1/2 inches), and of length/diameter (UD) ratio from about 100:1 to about 2000:1, preferably about 150:1 to about 2000:1, it being an advantage of the invention that good performance has been obtainable with preferred water-dispersible fiber of the invention with an UD ratio higher than we have considered satisfactory with prior art water-dispersible polyester fiber. For instance, machine manufacturers have generally recommended that the UD ratio not exceed 500:1, and many operators have considered even this figure unrealistically high. A suitable denier per filament is generally from about 0.5 to about 20 (about 0.55 to about 22 dtex). The coating is generally present in amount about 0.04 to about 1.0% of the weight of fiber (OWF%), it being an advantage that smaller amounts may generally be used than we have considered satisfactory according to the prior art.

There is also provided a process for preparing such water-dispersible polyester fiber as claimed in claim 10.

The coating is preferably cured on the filaments by heating the coated filaments, or the resulting staple fiber, if desired, to a temperature of about 100° to about 190° to improve durability.

The invention is further illustrated in the following Example, in which all parts and percentages are by weight, unless otherwise indicated, and OWF is (solids) "of weight of fiber". Reference is made to several measurements of yarn properties, such as tensile properties (tenacity and elongation-to break), which are measured according to the methods described in Frankfort et al. U.S. Patent No. 4,134,882. It will be understood that other conditions can be used e.g., other designs of orifice, such as are shown in the art.

### Example

The following fibers, Fiber A, a comparison of round cross section, and Fiber N, a fiber of the invention of cruciform cross section, were both spun from poly(ethylene terephthalate) of intrinsic viscosity 0.64, containing 0.3% Ti0₂ as a delusterant.

Fiber A was spun at 1600 ypm (1463 m/min) into filaments with conventional radial air quenching using a 900 hole spinneret, with round holes 0.015 inches (0.381 mm) in diameter and capillary length of 0.030 inches (0.762 mm), a 270°C block, and polymer throughput 68.2 pounds/hour (30.9 kg/hour). Denier per filament was 3.67 (4.04 dtex). Fiber A was then oriented by running over a set of feed rools at 29.3 ypm (26.8 m/min), followed by a set of draw rolls at 80.0 ypm (73.15 m/min), and delivered to a conveyer by puller rolls at 80.1 ypm (73.24 m/min). Between feed roll sections the filaments were treated in a 45°C water bath. Between feed and draw rolls the rope was sprayed with water at 98°C. Between draw and puller rolls a commercial water-dispersible coating (50/50 mixture of potassium salt of mono and diacid phosphate esters of lauryl alcohol/tallow alcohol ethoxylated with 25 moles of ethylene oxide) was applied. The filaments were then relaxed free in an oven at 150°C for 6 minutes.

Fiber N was produced in a similar manner to Fiber A except that 625 filaments of 3.22 dpf (3.54 dtexpf) and cruciform cross-section were spun through capillaries as shown in Figure 2, with block temperature 273°C, and throughput 42.9 pounds/hour (19.5 kg/hour). Roll speeds for the orientation were feed rolls 32.1 ypm, (29.4 m/min), draw rolls 80.2 ypm (73.3 m/min) and puller rolls 79.2 ypm (72.4 m/min), and a somewhat higher level of water-dispersible coating was used to offset approximately 57% higher surface area of the cruciform cross-section.

The properties of the drawn coated filaments are compared in Table 1.

Both types were cut to form water-dispersible fiber of 1/4, 3/8, 1/2 and 3/4 inch (6.35 mm, 9.53 mm, 12.70 mm, and 19.05 mm) cut lengths and were tested on an inclined wire Fourdrinier machine. Fibers were dispersed for three minutes in a small pulper at 0.75% consistency (kg, fiber per 100 kg. slurry, or furnish). The cylindrical pulper was approximately 3 feet (0.91 m) in diameter by 6 feet (1.83 m) deep. Fibers were then mixed with unrefined sulphite pulp to form a 50% polyester blend and diluted to 0.1 % consistency in a 10 cubic meter stock tank. This stock was further diluted in the headbox of the machine to 0.0143% consistency and formed into a 0.5 meter wide wet lay nonwoven fabric at 20 meters/minute. A spray of an acrylic binder. Acronyl 240D was spray applied at the end of the Fourdrinier wire. The fabric was then cured in a through air drier at 150°C. Finished fabric weight averaged 40 grams/square meter.

Dispersion quality can be judged by the uniformity of the fabric produced from a given sample. As cut length increases, the uniformity of the fabric can generally be expected to suffer significantly. However, great advantages can result from using a longer fiber because the fabric tear strength increases, for example. In practice, therefore, a fabric producer will generally wish to use the longest fiber that will meet his uniformity standards. Thus, a longer fiber with improved, or equivalent uniformity would be preferred.

The dispersion quality of fabrics from fibers A and N were rated as they were produced on the machine by observing the fabrics as the water drained from them on the Fourdrinier wires. Results of this comparison are in Table 2 and indicate good dispersion for the cruciform in spite of its 57% greater surface area.

Standard physical properties were measured for the set of fabrics at Herty foundation, Savannah, GA. Compared each time to Fiber A as 100%, Fiber N had the following average properties:

On balance, item N exhibited advantages in the important areas of higher permeability, opacity, bulk and tear strength compared to the control at equivalent tensile strength with a small reduction in stretch. The cover advantage is important because less fiber, can be used for a nonwoven fabric with similar performance characteristics, thereby saving materials cost. The fabrics of Item N also have an attractive flannel-like hand.

When used with the appropriate water-dispersible coating in appropriate amount, the cruciform cross-section fiber of the invention has given a fabric with surprisingly good dispersion uniformity, and the properties indicated.

From theoretical considerations, water-dispersible fibers of conventional round cross-section would have been expected to give more uniform dispersions, and, therefore, more uniform wet-laid fabrics. This is because the surface energy required to disperse a fiber (or other articles) is given by:
Energy=(Surface Tension) x (Dispersed surface area-Undispersed surface area).

The undispersed fiber exists in logs or clumps of many hundreds of fibers, most of which are on the inside of the logs. Therefore the undispersed surface area is negligible compared to the dispersed area; and the energy term can be expressed approximately as:
Energy=(Surface Tension) x (Number of fibers) x (Surface area of fiber).

This energy term describes both the energy required to disperse the fiber, and the free energy driving force for reagglomeration. Therefore, for any given coating, and fiber dpf, fibers with lower area would be expected to provide a more uniform dispersion, hence more uniform fabric. The minimum surface area per unit weight for a given fiber occurs when the cross-section is round, which would be expected, therefore, to be preferred.

Surprisingly, however, these cruciform fibers, in spite of about 60% greater surface area gave more uniform fabrics. Without limiting the invention in any theory, this may result from the fiber's hydrodynamic shape, which may more effectively use the energy available in the mixer shear field.

## Claims

1. Synthetic polymer fiber rendered water-dispersible by a coating promoting water-dispersibility, characterized in that the fibers are of cruciform cross-section.

2. Water-dispersible fiber as claimed in claim 1, of cut length from 5 to 90 mm, and wherein the length/diameter ratio is from 100:1 to 2000:1.

3. Water-dispersible fiber as claimed in claims 1 or 2, wherein the denier is from 0.5 to 20.

4. Water-dispersible fiber as claimed in any of claims 1 to 3, in the form of a package of cut fiber.

5. Polymer fibers of claim 1, in the form of a continuous filamentary uncrimped tow.

6. Fiber as claimed in any of preceding claims, characterised in that the synthetic polymer is polyester.

7. Polyester fiber according to claim 6, consisting essentially of poly(ethylene terephthalate).

8. Polyester fiber as claimed in claim 7, wherein the fiber is an essentially uncrimped poly(ethylene terephthalate) fiber, of cut length 5 to 90 mm, of length/diameter ratio 100:1 to 2000:1, and of denier 0.5 to 20, and an ethoxylated water-dispersing coating is present in amount 0.04 to 1.0% of the total weight of the fiber.

9. Polyester fiber according to claim 7, coated with a water-dispersing coating consisting essentially of a segmented copolyester of poly(ethylene terephthalate) repeat units and poly(oxyalkylene) groups derived from a poly(oxyalkylene) glycol having an average molecular weight in the range of 300 to 6000.

10. A process for preparing polyester fiber rendered water-dispersible by a coating promoting water-dispersibility, by melt-spinning the polyester into filaments, drawing the tow and cutting the filaments, characterized in that the polyester is spun into filaments of cruciform cross-section, the filaments are coated with a segmented synthetic copolyester of poly(ethylene terephthalate) repeat units and poly(oxyalkylene) groups derived from a poly(oxyalkylene) glycol having an average molecular weight in the range of 300 to 6,000, and cut to fibers of cut length from 5 to 90 mm.

11. A process as claimed in claim 10, wherein the filaments are coated with the copolyester in amount 0.04 to 1.0% of their weight.

12. A process as claimed in claims 10 or 11, wherein the coating is cured on the filaments by heating the coated filaments to a temperature of 100°C to 190°C.

## Patentansprüche

1. Synthetische Polymerfasern, die mittels eines Überzugs zur Verstärkung der Wasserdispergierbarkeit dispergierbar gemacht ist, dadurch gekennzeichnet, daß die Fasern einen kreuzförmigen Querschnitt haben.

2. Wasserdispergierbare Faser nach Anspruch 1 mit einer Schnittlänge von 5 bis 90 mm, bei der das Längen/Durchmesser-Verhältnis sich von 100:1 zu 2000:1 beläuft.

3. Wasserdispergierbare Faser nach Anspruch 1 oder 2, bei der der Titer 0,5 bis 20 den beträgt.

4. Wasserdispergierbare Faser nach einem der Ansprüche 1 bis 3, welche die Form eines Pakets aus Schnittfasern hat.

5. Polymerfasern nach Anspruch 1, die in Form eines endlosen, ungekräuselten Filamentkabels vorliegen.

6. Faser nach einem der vorangehenden Ansprüche, dadurch gekennzeichnet, daß das synthetische Polymer Polyester ist.

7. Polyesterfaser nach Anspruch 6, die im wesentlichen aus Poly(ethylenterephthalat) besteht.

8. Polyesterfaser nach Anspruch 7, bei der die Faser eine im wesentlichen ungekräuselte Poly(ethylenterephthalat)Faser mit einer Schnittlänge von 5 bis 90 mm, einem Verhältnis von Länge/ Durchmesser von 100:1 bis 2000:1 ist, und einen Titer von 0,5 bis 20 den hat, und bei der ein ethoxylierter wasserdispergierender Überzug in einer Menge von 0,04 bis 1,0% des Gesamtgewichts der Faser vorhanden ist.

9. Polyesterfaser nach Anspruch 7, die mit einem wasserdispergierenden Überzug beschichtet ist, der im wesentlichen aus einem segmentierten Copolyester aus Poly(ethylenterephthalat)-Wiederholungseinheiten und Poly(oxyalkylen)-Gruppen besteht, die von einem Poly(oxyalkylen)-glycol abgeleitet sind, das ein mittleres Molekulargewicht in der Größenordnung von 300 bis 6000 hat.

10. Verfahren zum Herstellen einer Polyesterfaser, die mittels eines Überzugs zur Förderung der Wasserdispergierbarkeit wasserdispergierbar gemacht ist, bei dem der Polyester zu Filamenten gesponnen, das Kabel verstreckt und auf Stapel geschnitten wird, dadurch gekennzeichnet, daß der Polyester un Filamenten mit kreuzförmigem Querschnitt gesponnen wird, die Filamente mit einem segmentierten synthetischen Copolyester aus Poly(ethylenterephthalat)Wiederholungseinheiten und Poly(oxyalkylen)-Gruppen beschichtet wird, die von einem Poly(oxyalkylen)-glycol abgeleitet sind, das ein mittleres Molekulargewicht in der Größenordnung von 300 bis 6000 hat, und diese zu Fasern mit einer Schnittlänge von 5 bis 90 mm geschnitten werden.

11. Verfahren nach Anspruch 10, bei dem die Filamente mit Copolyester in einer Menge von 0,04 bis 1,0 Gew.-% beschichtet sind.

12. Verfahren nach Anspruch 10 oder 11, bei dem die Beschichtung auf den Filamenten durch Erwärmung der beschichteten Filamente auf eine Temperatur von 100°C bis 190°C ausgehärtet wird.

## Revendications

1. Fibre de polymère synthétique rendue dispersible dans l'eau par un revêtement favorisant à la dispersibilité dans l'eau, caractérisée en ce que les fibres sont de section transversale cruciforme.

2. Fibre dispersible dans l'eau telle que revendiquée dans la revendication 1, d'une longueur de coupe de 5 à 90 mm, et dont le rapport longueur/diamètre est de 100:1 à 2000:1.

3. Fibre dispersible dans l'eau telle que revendiquée dans la revendication 1 ou 2, dont le denier est de 0,5 à 20.

4. Fibre dispersible dans l'eau telle que revendiquée dans l'une quelconque des revendications 1 à 3, sous la forme d'un paquet de fibre coupée.

5. Fibres de polymère de la revendication 1, sous la forme d'un câble non frisé de filaments continus.

6. Fibre telle que revendiquée dans l'une quelconque des revendications précédentes, caractérisée en ce que le polymère synthétique est un polyester.

7. Fibre de polyester selon la revendication 6, essentiellement constituée de poly(téréphtalate d'éthylène).

8. Fibre de polyester telle que revendiquée dans la revendication 7, dans laquelle la fibre est une fibre de poly(téréphtalate d'éthylène) essentiellement non frisée ayant une longueur de coupe de 5 à 90 mm, un rapport longueur/diamètre de 100:1 à 2000:1 et un denier de 0,5 à 20, et un revêtement éthoxylé de dispersion dans l'eau esat présent à raison de 0,04 à 1.0% du poids total de la fibre.

9. Fibre de polyester selon la revendication 7, revêtue d'un revêtement de dispersion dans l'eau essentiellement constitué d'un copolyester séquencé de motifs répétés poly(téréphtalate d'éthylène) et de groupes poly(oxyalkylène) dérivés d'un poly(oxyalkylène)-glycol ayant un poids moléculaire moyen compris dans la gamme de 300 à 6000.

10. Un procédé pour fabriquer une fibre de polyester rendue dispersible dans l'eau par un revêtement favorisant la dispersibilité dans l'eau, par filage à l'état fondu du polyester en filaments, étirage du câble et coupe des filaments, caractérisé en ce que le polyester est filé en filaments de section transversale cruciforme, les filaments sont revêtus avec un copolyester, synthétique séquencé de motifs répétés poly(téréphtalate d'éthylène) et de groupes poly(oxyalkylène) dérivés d'un poly(oxyalkylène)-glycol ayant un poids moléculaire moyen compris dans la gamme de 300 à 6000, et coupés en fibres d'une longueur de coupe de 5 à 90 mm.

11. Un procédé tel que revendiqué dans la revendication 10, dans lequel les filaments sont revêtus par le copolyester à raison de 0,04 à 1,0% de leur poids.

12. Un procédé tel que revendiqué dans la revendication 10 ou 11, dans lequel le revêtement est durci sur les filaments par chauffage des filaments revêtus à une température de 100°C à 190°C.
